

# UNITED STATES PATENT OFFICE.

MILTON C. WHITAKER, OF NEW YORK, N. Y., ASSIGNOR TO U. S. INDUSTRIAL ALCOHOL CO., A CORPORATION OF WEST VIRGINIA.

## INTERNAL-COMBUSTION-ENGINE FUEL.

1,420,006.

Specification of Letters Patent. Patented June 20, 1922.

No Drawing.

Application filed November 12, 1919. Serial No. 337,395.

To all whom it may concern:

Be it known that I, MILTON C. WHITAKER, a citizen of the United States, residing at New York, in the county of New York and State of New York, have invented a certain new and useful Improvement in Internal-Combustion-Engine Fuel, of which the following is a specification.

My invention relates particularly to fuels 10 designed to be used in aeroplane motors, but is applicable for use in internal combustion motors of all kinds used in flying or for other purposes.

The object of my invention is to provide 15 a fuel which is especially adapted for use in aeroplanes, although it is also applicable for use in internal combustion engines in general.

It is necessary that fuels which are to be 20 used in aeroplane motors shall have great dependability, inasmuch as any uncertainty in the operation of the aeroplane by reason of variability in the character of the fuel or failure of the fuel to perform its intended 25 work, may bring about disastrous consequences.

For this reason, it is desirable to avoid 30 using in such fuels large percentages of petroleum products, inasmuch as commercial petroleum products do not ordinarily have a constant composition, and are usually comprised of varying quantities of a number of different constituents.

It is, therefore, the object of my invention 35 to provide a motor fuel avoiding these disadvantages and taking into account the circumstances above referred to.

Still a further object of my invention is to 40 provide fuels of the above character by the use of ketones but especially higher ketones, that is to say, ketones other than acetone.

Further objects of my invention will appear from the detailed description thereof contained hereinafter.

While my invention is capable of being 45 carried out in different ways, for the purpose of illustration I shall describe only certain ways of carrying out the same herein.

For example, a fuel made in accordance 50 with my invention may be comprised of—  
35 parts by volume of acetone,  
25 parts by volume of alcohol,  
5 parts by volume of ethyl acetate,

17 $\frac{1}{2}$  parts by volume of kerosene, 55  
17 $\frac{1}{2}$  parts by volume of gasoline.

Another example is:

35 parts by volume of methyl-ethyl-ketone, 60  
25 parts by volume of alcohol,  
5 parts by volume of ethyl acetate,  
17 $\frac{1}{2}$  parts by volume of kerosene,  
17 $\frac{1}{2}$  parts by volume of gasoline.

Another example is: 65  
35 parts by volume of diethyl ketone,  
25 parts by volume of alcohol,  
5 parts by volume of ethyl acetate,  
17 $\frac{1}{2}$  parts by volume of kerosene,  
17 $\frac{1}{2}$  parts by volume of gasoline.

The above compositions may be varied to 70 a considerable extent. For example, the kerosene and gasoline may be substituted by the same total quantity of a single petroleum distillate, such for example as gasoline or kerosene. Instead of ethyl acetate, I 75 may use any one of a number of esters, as for example methyl butyrate, ethyl butyrate, methyl acetate, butyl acetate or amyl acetate, all of which are volatile esters or still other esters could be used as for example, 80 castor oil.

Also other alcohols may be used instead of ethyl alcohol, such for example as methyl alcohol, butyl alcohol or amyl alcohol.

While I have described my invention 85 above in detail, I wish it to be understood that many changes may be made therein without departing from the spirit thereof.

I claim:

1. A fuel comprising a light hydrocarbon, 90 an alcohol, diethyl ketone, and an ester.

2. A fuel comprising approximately equal proportions of a ketone, an alcohol, and a light petroleum distillate, with a smaller proportion of a volatile ester. 95

3. A fuel comprising a light hydrocarbon, alcohol, diethyl ketone and ethyl acetate.

4. A fuel comprising about 35% ketone, about 25% alcohol, about 35% petroleum distillate, and about 5% of an ester. 100

5. A fuel comprising about 35% diethyl ketone, about 25% alcohol, about 35% petroleum distillate, and about 5% ethyl acetate.

In testimony that I claim the foregoing, I have hereunto set my hand this 6th day 105 of November, 1919.

MILTON C. WHITAKER.